

## [54] CONVERSION OF PIG IRON INTO STEEL

[75] Inventor: Paul Emile Nilles, Embourg, Belgium

[73] Assignee: Centre de Recherches Metallurgiques, Brussels, Belgium

[22] Filed: Nov. 3, 1972

[21] Appl. No.: 303,357

## [30] Foreign Application Priority Data

Nov. 3, 1971 Belgium ..... 774886

[52] U.S. Cl. .... 75/60; 75/52

[51] Int. Cl. .... C21c 5/32

[58] Field of Search ..... 75/60, 52

## [56] References Cited

## UNITED STATES PATENTS

|           |         |                |       |
|-----------|---------|----------------|-------|
| 1,793,153 | 2/1931  | Becket .....   | 75/60 |
| 2,855,293 | 10/1958 | Savard .....   | 75/60 |
| 2,918,365 | 12/1959 | Kanamori ..... | 75/60 |
| 3,015,554 | 1/1962  | Rummel .....   | 75/60 |

|           |         |                |       |
|-----------|---------|----------------|-------|
| 3,079,249 | 2/1963  | Moustier ..... | 75/60 |
| 3,330,645 | 7/1967  | Moustier ..... | 75/60 |
| 3,556,773 | 1/1971  | Grenfell ..... | 75/52 |
| 3,706,549 | 12/1972 | Knuppel .....  | 75/60 |

Primary Examiner—L. Dewayne Rutledge

Assistant Examiner—Peter D. Rosenberg

Attorney, Agent, or Firm—Holman &amp; Stern

## [57] ABSTRACT

A refining process for converting pig iron into steel wherein at least one tuyere is mounted in the side wall on the converter and the tuyere has an inner conduit and an outer conduit. Substantially pure oxygen is injected through the inner conduit and a protective fluid is injected through the outer conduit. The axis of the tuyere is inclined towards the bottom of the converter so that the injected oxygen creates rotational movement in the molten metal so as to better distribute the oxygen throughout the melt and control the decarbonization of the converter. The tuyere in the side wall is mounted at the level of the zone occupied by the slag.

6 Claims, 3 Drawing Figures





FIG. 1



FIG. 2

## CONVERSION OF PIG IRON INTO STEEL

## BACKGROUND OF THE INVENTION

The present invention relates to a refining process for the conversion of pig iron into steel.

It is known that the problem of the life of the bottom of an oxygen-blown converter has been solved by the use, for the injection of industrially pure oxygen beneath the surface of the metallic bath, of tuyeres comprising two concentric conduits located either in the bottom or in the side wall beneath the surface of the metallic bath, the central conduit serving for the blowing-in of pure oxygen, the peripheral conduit serving for the blowing in of liquid or gaseous protective fluid. This solution is generally considered as satisfactory.

However, it has been confirmed that, particularly with regard to injection through the bottom, actual control of the evolution of the slag composition during refining is achieved with difficulty. As is known, this control is linked with the possibility of controlling the foaming of the slag, the decarburization rate, and the distribution of the oxygen between the hot metal and the slag.

## SUMMARY OF THE INVENTION

The present invention provides a refining process in which, by means of one or more tuyeres comprising two coaxial tubes and located in the wall of a converter, above the upper level of the hot metal, technically pure oxygen is injected into the metal bath through the central tube of the tuyeres and then a liquid and/or gaseous protective fluid is injected through the peripheral conduit of the tuyeres, the tuyeres being inclined towards the bottom of the converter.

The oxygen and the protective fluid may advantageously be injected through one or more such tuyeres in the wall of the converter at the level of the zone occupied by the slag, which enables the appearance of the reactive character of the slag to be accelerated.

Owing to the possibility of placing the oxygen directly in contact with the slag and metal, the present process has the important advantage of allowing an easy distribution of the oxygen between the metal and the slag and consequently the control of the decarburization rate; furthermore, inclination of the tuyere enables wear of the refractories in the side wall opposite the tuyere to be avoided.

It has been confirmed that with the present process it is also possible to avoid the formation of metallic heads on the periphery of the tuyeres within the converter; such heads constitute a handicap to the processes in which the injection of oxygen is made beneath the surface of the hot metal.

The diameter of the tuyere as well as the rate of flow of oxygen and protective fluid are preferably arranged to be adjustable and controllable, in order to accelerate the refining of the pig iron, particularly by helping to rapidly form a fluid reactive slag.

Each injection may advantageously be effected along an axis inclined towards the bottom of the converter and located in a diametrical plane of the converter, which results in producing in the metal a double rotational movement at one and the same time in a vertical plane and in a horizontal plane, which produces excellent mixing of the hot metal and thorough decarburization.

The injection can be carried out by means of a single tuyere, directed towards the bottom of the converter, the direction of the jet of oxygen not however passing through the axis of the converter.

5 The injection may be carried out simultaneously on different levels, namely above the level of the slag and into the slag, their direction not passing through the longitudinal axis of the converter. By judiciously selecting the speeds and rates of flow to the different injection tuyeres, a differential rotational movement between the metal and the slag is achieved, which enables the physico-chemical exchanges at the slag/metal interface to be increased, and therefore accelerates decarburization.

10 15 The rotational movements imparted to the slag and metal are judiciously controlled by the arrangement of the tuyeres in the wall of the converter. For this purpose, according to requirements, the tuyeres can be arranged to be orientated in the same sense in relation to the axis of the converter or in the opposed sense, whether side by side or spaced, in the wall of the converter all around its periphery.

20 It is within the scope of the present invention to place one or several pulverulent materials, preferably slagging materials, such as for example lime, in suspension in the oxygen.

25 The protective fluid is advantageously composed of a gaseous or liquid hydrocarbon.

## BRIEF DESCRIPTION OF THE DRAWINGS

FIG. 1 is a vertical cross-section of a converter according to the instant invention; and

25 30 FIGS. 2 and 3 are simplified horizontal cross-sections of the outside wall of the converter showing two embodiments of the invention.

## DETAILED DESCRIPTION OF THE EMBODIMENTS

According to FIG. 1, tuyere 1 has an inner tube 2 for 40 the blowing of oxygen and this tube 2 is surrounded by a concentric tube 3 through which a cooling medium is injected. This tuyere 1 is inserted in a side wall 4 of a converter 5 and the longitudinal axis 6 of this tuyere 1 is inclined towards the converter bottom with the jet of oxygen directly impinging on slag 7, molten metal 8 being underneath.

45 The angle of inclination of the tuyere is  $\alpha$  and is the angle made by the longitudinal axis 6 of the tuyere with a horizontal plane 9 passing through a point 10 where this longitudinal axis 6 enters the converter, when the converter is stationary with its longitudinal axis 12 in vertical position.

50 FIG. 2 shows the tuyere 1 with its longitudinal axis 6 inclined towards the bottom of the converter and located in the diametrical plane of the converter. Such a location results in producing in the metal a double rotational movement (arrows 13 and 14) at one and the same time. This movement also takes place in a vertical plane and in a horizontal plane because of the inclination  $\alpha$  of the tuyere towards the metallic bath.

55 60 The jet of oxygen with cooling medium impinges the molten metal and produces two force components: one vertical (arrow 15, FIG. 1) and one horizontal (arrow 16, FIG. 1).

65 FIG. 3 shows the tuyere 1 having a longitudinal axis 6 which does not intersect longitudinal axis 12 of the converter. The direction of this axis 6 many be defined

by a distance 17 between axis 6 and axis 12. Such a direction enables a rotational movement (arrow 18) in the metal and in the slag to be achieved. In the case of several tuyeres located at different levels, a differential rotational movement between the metal and the slag may be achieved by judiciously selecting the speeds and rates of flow to different injection tuyeres.

I claim:

1. A refining process for the conversion of pig iron into steel in a converter wherein the molten metal is agitated by blown oxygen so as to better distribute the oxygen throughout the melt and control the decarburization, the converter having a bottom, a side wall, and at least one tuyere in the side wall, the tuyere comprising an inner conduit and an outer conduit surrounding the inner conduit, the process including the steps of injecting substantially pure oxygen through said inner conduit onto the molten metal in the converter, and injecting a protective fluid through the outer conduit, the tuyere opening into the converter through the sidewall at the level of the zone occupied by slag and the axis of the tuyere being inclined towards the converter bot-

tom to create rotational movement of the molten metal.

2. A process as claimed in claim 1, in which the axis of the tuyere is directed along a line contained in a diametrical plane of the converter.

3. A process as claimed in claim 1, in which only one tuyere is used, the axis of the tuyere being directed towards the converter bottom along a line which does not intersect the converter axis.

10 4. A process as claimed in claim 1, in which two tuyeres are used, one opening into the converter above the slag layer and the other opening into the slag layer, the axis of each tuyere being directed along a line which does not intersect the axis of rotation of the converter, the speed and flow rate of the materials injected through the tuyere being such that the molten metal and the slag rotate at different speeds.

15 5. The process as claimed in claim 1, in which powdery material is in suspension in the injected oxygen.

20 6. The process as claimed in claim 1, in which the protective fluid is a hydrocarbon.

\* \* \* \* \*

25

30

35

40

45

50

55

60

65